

## UNITED STATES PATENT OFFICE

2,118,839

TREATMENT OF ARTIFICIAL FILAMENTS,  
THREADS, YARNS, FABRICS, AND THE  
LIKE

Henry Dreyfus, London, England

No Drawing. Application January 30, 1935, Se-  
rial No. 4,084. In Great Britain February 28,  
1934

9 Claims. (Cl. 28—1)

This invention relates to improvements in the treatment of artificial filaments, threads, yarns, fabrics and the like, and is more particularly directed to the treatment of cellulose ester and ether materials for the purpose of obtaining fabrics or other textile materials of improved handle.

In U. S. applications S. Nos. 746,134 filed 29th September, 1934, and 746,135 filed 29th September, 1934, and S. Nos. 4,086 and 4,085 both filed January 30, 1935, processes are described wherein inter alia yarns of cellulose acetate or other esters or ethers of cellulose are subjected to treatment with steam or hot water, particularly under conditions of tension which bring about a stretching of the material, so as to produce crêpe fabrics, the treatment with the steam or hot water taking place before the application of the crêpe twist or during a single stage crêpe twisting operation or during any of the stages of a di- or multi-stage crêpe twisting operation or between any two stages of a di- or multi-stage crêpe twisting operation. Further, in U. S. applications S. Nos. 4,510 and 4,511 both filed February 1, 1935, processes are described for stretching yarns or other materials of cellulose acetate or other cellulose esters or ethers with the assistance of steam or hot water.

I have now found that the handle of materials treated by any of the above processes is substantially improved by subjecting the materials to a mild treatment with solvents, swelling agents or softening agents for the substance of the material under treatment. Preferably the treatment is such that the solvent, swelling agent or softening agent does not completely penetrate the materials so that its action is not homogeneous and may be extremely superficial. Thus, the outer layers only may be acted upon by the solvent or other softening agent.

The action of the softening agent may be restricted to the outer layers only of the filaments or other materials under treatment in any suitable way. For example the agent may be applied in small quantities only so that it does not penetrate to the core. Alternatively or in addition, and this is the most important method, the time factor may be utilized to prevent the softening agent from penetrating completely. Generally I prefer to use agents which are either non-volatile and/or have a low softening power. The agents of high softening power which have comparatively low volatility appear to be less rapid in penetrating the substance of the material, so that their action may be arrested by removal of

the softening agent before complete penetration has taken place. Similarly, substances which are volatile but which have only a low softening power for the material under treatment may be used and may be removed sufficiently rapidly by evaporation to avoid complete penetration. However, washing of the softening agent from the material is the most effective method of limiting the action of the agent to the outer layers of the material.

As indicated it is advisable, except when employing substances of low penetrating power, to employ only a limited quantity of the softening agent. Thus, the solvent or softening agent may be applied in the vapour state, though even here it is advisable to treat the materials only for a short time.

The process of the invention may be applied to the treatment of filaments, threads, yarns or other materials made of or containing cellulose derivatives, as for instance cellulose acetate, and particularly acetone-soluble cellulose acetate, cellulose formate, cellulose propionate or butyrate or other esters or mixed esters, and methyl, ethyl, butyl and benzyl celluloses, or other cellulose ethers or mixed ethers and also mixed ether-esters, for instance ethyl cellulose acetate and oxyethyl cellulose acetate. Examples of the swelling agents which may be employed are thiocyanates, zinc chloride, lower aliphatic acids, for example lactic acid and the like, ketones, for instance methyl-ethyl ketone, esters, for instance ethyl lactate, diethyl tartrate and the like, the ethers, including cyclic ethers, esters and ether-esters of olefine or polyolefine glycols or glycerine, e. g. glycol monoacetate, methyl or ethyl glycol monoacetate and the like, chlorinated hydrocarbons, as for instance tetrachlorethane, trichlorethylene, dichlorethylene and the like, phenols, certain alcohols, e. g. ethyl alcohol, etc. Moreover, liquids which at normal temperatures have no softening action or substantially no softening action but which at higher temperatures have such action may be employed at temperatures above atmospheric temperature. Examples of such liquids are glycols, glycerine and Turkey red oil.

Thus for example a very short treatment with cold dilute formic acid or acetic acid followed by removal of the softening agent is very effective for the purpose of the present invention since by such treatment the handle of the goods is substantially improved, and in particular they are much softer to the touch. Thus for instance the goods may be padded with a 10% aqueous solu-

tion of formic or acetic acid, given a short air run, and the acid immediately washed off, for example by thorough washing in water at a temperature of the order of 60 to 80° C. The speed 5 of the materials and the length of passage through the padding mangle and the length of the air run may be adjusted so that the total time during which the materials are in contact with the acid is less than a minute, and is preferably half a minute or even less. Alternatively, 10 less powerful softening agents may be employed, as for example a 70 to 80% aqueous solution of methylated spirit or an 80% solution of tetrachlorethane in toluene. In all cases however it is desirable to limit the time during which the 15 materials are in contact with the softening agents so that penetration is limited to the outer layers only.

The treatment in accordance with the present 20 invention may be so conducted that the final filaments are lustrous in appearance or have a medium or quite dull lustre. If the treatment is carried out so that on removal of the softening medium the concentration of the solvent in 25 the medium decreases, then a dull lustre may result from the present treatment, while if the concentration remains about the same or increases, then the lustre may be maintained or even increased.

30 The treatment in accordance with the present invention may be carried out so that a slight stretch is applied to the filaments during the solvent treatment.

The solvent treatment may be applied to the 35 materials at any suitable stage after they have been subjected to the stretching and/or crêpe twisting in the presence of steam, hot water or the like. Thus the solvent treatment may be applied before the yarn is formed into fabrics. 40 Preferably, however, the solvent treatment may be applied subsequent to fabric formation and subsequent to the development of the crêpe figure. The invention does, however, include the solvent treatment of materials which have been 45 stretched in the presence of steam or hot water or similar agents quite apart from the production of crêpe fabrics.

The following examples illustrate without in any way limiting the invention:—

50

*Example 1*

A fabric comprising cellulose acetate yarns in the warp and weft, the weft yarns having been treated with steam and given a crêpe twist as 55 described in U. S. applications S. Nos. 746,134 and 746,135, is scoured or otherwise treated to produce a crêpe figure. The crêpe fabric resulting is padded with 10% aqueous formic or acetic acid. After about 30 seconds the acid is removed 60 from the fabric by thoroughly and rapidly washing with water at a temperature of about 70° C.

*Example 2*

A dry spun cellulose acetate yarn is stretched 65 to about 300 or 400% of its original length in the presence of steam or hot water as described in U. S. applications S. Nos. 4,510 and 4,511 and is then carefully dried. The dry yarn is then immersed for 2 minutes at room temperature in a bath consisting of 80% by volume of tetrachloroethane and 20% of toluene. After removal from the bath the yarn is washed with toluene and dried.

*Example 3*

A dry spun cellulose acetate yarn is stretched

as described in Example 2 and, while still wet, is passed at a speed of 20 metres per minute over a heated roller running in diethylene glycol at a temperature of 105° C. The yarn is then passed over a wick, pad or other wiping device, 5 washed substantially free from diethylene glycol and dried.

*Example 4*

The cellulose acetate crêpe fabric of Example 10 1 is subjected to the mild softening treatment there described except that in place of the acid solutions a 10% solution of glycol monoacetate is employed.

What I claim and desire to secure by Letters 15 Patent is:—

1. Process for improving the handle of textile materials comprising cellulose derivative yarns which have been subjected to a crepe twisting operation in the presence of steam or hot water, 20 which comprises treating the materials with a swelling agent for the cellulose derivative for a very short period, and removing the agent from the materials after it has penetrated the outer layers only of the filaments contained in the 25 yarns.

2. Process for improving the handle of textile materials comprising cellulose acetate yarns which have been subjected to a crepe twisting operation in the presence of steam or hot water, 30 which comprises treating the materials with a swelling agent for the cellulose acetate for a very short period, and removing the agent from the materials after it has penetrated the outer layers only of the filaments contained in the 35 yarns.

3. Process for improving the handle of textile materials comprising cellulose acetate yarns which have been subjected to a crepe twisting operation in the presence of steam or hot water, which comprises subjecting the filaments 40 contained in the yarns to the action of a relatively non-volatile swelling agent for the cellulose acetate for a few minutes so that penetration is limited to the outer layers only and then removing the swelling agent.

4. Process for improving the handle of textile materials comprising cellulose acetate yarns which have been subjected to a crepe twisting operation in the presence of steam or hot water, which comprises subjecting the filaments contained in the yarns to the action of an agent having only a slight swelling action on the cellulose acetate for a period less than two minutes so that penetration is limited to the outer layers only and then removing the swelling agent.

5. Process for improving the handle of textile materials comprising cellulose acetate yarns which have been subjected to a crepe twisting operation in the presence of steam or hot water, which comprises treating the materials with a 60 relatively non-volatile agent having at least a softening action on the cellulose acetate for a very short period, and removing the agent from the materials after it has penetrated the outer layers only of the filaments contained in the 65 yarns.

6. Process for improving the handle of textile materials comprising cellulose acetate yarns which have been subjected to a crepe twisting operation in the presence of steam or hot water, which comprises treating the materials with an 70 agent having only a slight swelling action on the cellulose acetate for a very short period, and removing the agent from the materials after it has penetrated the outer layers only of the filaments contained in the 75 yarns.

7. Process for improving the handle of textile materials comprising cellulose acetate yarns which have been subjected to a crepe twisting operation in the presence of steam or hot water, which comprises treating the materials with a dilute lower fatty acid in the cold for a period of less than one minute, and then washing the materials free from the acid.

8. Process for improving the handle of textile materials comprising cellulose acetate yarns which have been subjected to a crepe twisting operation in the presence of steam or hot water, and of textile materials comprising cellulose acetate yarns which have been stretched in the presence of steam or hot water, which comprises treating the materials with a dilute solution of a chlorinated

hydrocarbon having at least a strong swelling action on the cellulose acetate for a short period so that penetration is limited to the outer layers only, and then removing the solution from the materials.

9. Process for improving the handle of textile materials comprising cellulose acetate yarns which have been subjected to a crepe twisting operation in the presence of steam or hot water, which comprises treating the materials with a composition having a swelling action on the cellulose acetate and comprising a glycol ester of a lower fatty acid, and removing the composition by washing after it has penetrated the outer layers only of the filaments contained in the yarns.

HENRY DREYFUS.

CERTIFICATE OF CORRECTION.

Patent No. 2,118,839.

May 31, 1938.

HENRY DREYFUS.

It is hereby certified that error appears in the printed specification of the above numbered patent requiring correction as follows: Page 2, second column, lines 61 and 62, claim 5, for the words "agent having at least a softening action on" read swelling agent for; page 3, first column, lines 12 to 15 inclusive, claim 8, strike out the words and comma "and of textile materials comprising cellulose acetate yarns which have been stretched in the presence of steam or hot water,"; and that the said Letters Patent should be read with this correction therein that the same may conform to the record of the case in the Patent Office.

Signed and sealed this 2nd day of August, A. D. 1938.

(Seal)

Leslie Frazer,  
Acting Commissioner of Patents.